

**1**

2,830,950

**LUBRICATING COMPOSITIONS**

Clarence E. Rannefeld, Pensacola, Fla., assignor to Continental Oil Company, Ponca City, Okla., a corporation of Delaware

No Drawing. Continuation of application Serial No. 295,338, June 24, 1952. This application June 18, 1954, Serial No. 437,883

2 Claims. (Cl. 252—33.4)

This application is a continuation of my co-pending application, Serial No. 295,338, filed June 24, 1952, now abandoned.

This invention relates to lubricating compositions comprising a base oil of vegetable or mineral origin which may also contain small amounts of detergents, corrosion inhibitors, reserve alkalinity agents, and the like as additives. More particularly, the invention relates to heavy duty crankcase type lubricating oil compositions for use in diesel engines and the like which compositions comprise a major proportion of a mineral lubricating oil and minor amounts of an oil soluble detergent and/or an oxidation and corrosion inhibitor and as a reserve alkalinity agent a minor proportion of the barium salt of hydroabietyl alcohol.

Mixtures of dehydroabietyl alcohol, dihydroabietyl alcohol, and tetrahydroabietyl alcohol together with a small proportion of esters of hydrogenated rosin and hydrocarbons are available commercially under the trade-mark brand name "Abitol" by Hercules Powder Company of Wilmington, Delaware. For convenience the material is hereinafter referred to as hydroabietyl alcohol although it is believed to be comprised essentially of a mixture of hydrogenated abietyl alcohols containing a non-alcohol fraction amounting to about 13 to 15 percent. The alcohol mixture is thought to be made up of about 15 percent dehydroabietyl alcohol, about 40 percent dihydroabietyl alcohol, and the balance, about 45 percent, tetrahydroabietyl alcohol. The non-alcohol fraction varies with the saponification number but will average about 3 to 8 percent of the total mixture in the form of esters such as methyl esters of hydrogenated rosin and the remainder is similar to the hydrocarbon fractions occurring in hydrogenated rosin. Although the commercial product is most readily available at this time, it is apparent that the use of purer dehydroabietyl alcohol, dihydroabietyl alcohol, and tetrahydroabietyl alcohol, either alone or in admixture, in the preparation of alcoholates for addition to motor oils, is included within the scope of this invention.

The particular improvement of this invention resides in the addition to a lubricating oil of a barium salt of this hydroabietyl alcohol for the purpose of increasing the so-called "alkaline reserve" of the oil. The function of such materials is to neutralize acidity which is formed in the oil during use or in some manner to counteract the development of corrosive conditions formed in the oil during use.

The object of this invention is therefore to provide an improved lubricating oil composition having a high alkaline reserve content.

In preparing the improved oil of this invention, the barium salt of hydroabietyl alcohol was prepared by

**2**

mixing a portion of hydroabietyl alcohol in 170 S. S. U. pale oil with a substantial excess of barium oxide. The mixture was stirred under a blanket of an inert gas at 205–225° C. for several hours and filtered. The resulting barium alcoholate had a high base number and was oil soluble.

Lubricating compositions were then compounded by incorporating a small amount of barium hydroabietyl alcoholate prepared as above in a mineral oil containing a small proportion of an oil soluble detergent and a sulfur-containing corrosion inhibitor. These oil blends were found to be highly basic and, upon test runs in internal combustion engines, were found to materially decrease the deposits, particularly varnish, upon the pistons as compared with similar compositions not containing the alcoholate.

Although it is contemplated that the barium hydroabietyl alcoholate may be incorporated in lubricating oil compositions in amounts ranging from as little as 0.1 percent to as much as 10 percent, it has been found that for most satisfactory results amounts ranging from about 3 to 6 percent by weight should be employed. While either calcium diwaxbenzene sulfonate or barium diwaxbenzene sulfonate is shown as the detergent in each of the following examples, it will be readily apparent that other oil soluble detergents may also be used. Such detergents may include, by way of example, any of the following: Alkali and alkaline earth metal salts of (1) petroleum sulfonic acids obtained from the sulfuric acid treatments of kerosenes, distillate, light oil, wax distillate, or lube oil stocks, or sulfonic acids from the sulfonation of cracking cycle stocks, gas oil cycle stocks, hydroformer or cycloversion stocks, lube oil solvent extracts from cresol, phenol, Duosol, furfural, nitrobenzene, or Chlorex extraction of lube oil neutrals, bright stocks, or cylinder stocks, or the above compounds having preferably long chain alkyl substituents as alkylative condensation products of the above; (2) naphthenic acids of mineral origin obtained from kerosene, gas oil, distillate fuel, coal tar, lube oil, and similar stocks by caustic extraction, basic solvent extraction, or the like; (3) organic carboxylic acids such as barium cetyl benzoate, calcium dioctyl acetyl salicylate, strontium alpha-chloro-phenyl stearate, calcium monochlorstearate, zinc cetyl petrex, calcium octyl petrex, tin amyl-phenyl stearate, and the like; and (4) oil soluble alkyl phenols and naphthols such as calcium dioxyphenol, sodium nonyl naphtholate, barium diamyl phenol, potassium diwax-alkylated phenol, strontium dinonyl phenol, and the like. While the detergent may be present in amounts varying from about 1 to 10 percent, it is preferred to use between about 2 and 5 percent.

Any one of several sulfur-containing corrosion inhibitors may be used as indicated in the examples. In addition to those specifically mentioned, such other sulfur-bearing compounds may be used as: (1) phosphorus sulfide-hydrocarbon reaction products such as phosphorus pentasulfide treated octadecene, phosphorus trisulfide treated cetene, phosphorus pentasulfide treated propylene polymers, phosphorus pentasulfide treated terpenes, phosphorus pentasulfide treated wax distillate and gas oil olefins, phosphorus pentasulfide treated oil oxidation residues, and the like; (2) phosphorus sulfide-organic hydroxy reaction products such as phosphorus sulfide treated terpineol, phosphorus sulfide treated cyclohexanol, phosphorus sulfide treated alkyl substituted cyclohexanols, phosphorus sulfide treated tall oil alcohols,

## 3

phosphorus sulfide treated alkyl substituted naphthols, phosphorus sulfide treated alkyl substituted phenols, phosphorus sulfide treated cardanol, phosphorus sulfide treated oleyl alcohol, and the like; (3) phosphorus sulfide treated fatty acid esters such as phosphorus sulfide treated methyl oleate, phosphorus sulfide treated chlorinated methyl oleate, phosphorus sulfide treated methyl linoleate, phosphorus sulfide treated butyl ricinoleate, phosphorus sulfide treated esters of corn oil fatty acid, phosphorus sulfide treated esters of menhaden oil fatty acid, and the like; (4) sulfur and phosphorus sulfide treated compounds of the above groups particularly compounds having at least one sulfur or a phosphorus sulfide reactive olefin grouping or a phosphorus sulfide reactive hydroxy grouping or both such as sulfur and phosphorus sulfide treated oleic acid, sulfur and phosphorus sulfide treated butyl ricinoleate, sulfur and phosphorus sulfide treated 12-hydroxy stearic acid, and the like; (5) sulfurized compounds and synthetic sulfides prepared by the action of elemental sulfur on the organic compounds of group (1) about or on the sulfur reactive compounds, particularly mono-olefinic compounds, of groups (2), (3), and (4) above such as sulfur chloride condensed cetyl phenol, sulfur chloride condensed nonyl naphthal, sulfur dichloride condensed waxylated phenol, sulfur dichloride condensed diethyl phenol, dioctadecyl sulfide and/or disulfide, and the like.

In addition to the above materials, the alkali metal, alkaline earth metal, and non-catalytic heavy metal salts of each or any of the above comprising the neutralized or partially neutralized phosphorus sulfide or sulfide reaction products may be used. The inhibitor should be added in amounts such that from 0.1 to 0.35 percent sulfur will be present in the composition.

The preparation of the barium salt of hydroabietyl alcohol will now be described in detail by means of the following example.

In each of two 5-liter, 3-necked, flasks were placed 1,500 grams hydroabietyl alcoholate ("Abitol"), 1,765 grams of 170 pale oil, and 675 grams barium oxide. The barium oxide used was 100 percent in excess of the amount theoretically required. These materials were thoroughly mixed and the mixture was then stirred under a blanket of natural gas at 205-225° C. for 6 hours. The material from each batch was then filtered through diatomaceous earth. The base number of the first was 74.5 and of the other 75.7. The two batches were then combined with a portion of a third batch prepared in the same manner and the composite mixture of 16.67 pounds had a base number of 75.7. This resulting barium hydroabietyl alcoholate was then blended with a mineral S. A. E. 30 lubricating oil containing small amounts of calcium diwaxbenzene sulfonate and sulfur as phosphorus pentasulfide treated wax olefins as shown in the following examples:

## I

3 percent calcium diwaxbenzene sulfonate  
0.15 percent sulfur as phosphorus pentasulfide treated wax olefin  
3.58 percent barium hydroabietyl alcoholate  
Balance—mineral lubricating oil

## II

3 percent calcium diwaxbenzene sulfonate  
0.15 percent sulfur as phosphorus pentasulfide treated wax olefin  
3.93 percent barium hydroabietyl alcoholate  
Balance—mineral lubricating oil

## III

3 percent calcium diwaxbenzene sulfonate  
0.15 percent sulfur as phosphorus pentasulfide treated wax olefin

## 4

4.21 percent barium hydroabietyl alcoholate  
Balance—mineral lubricating oil

## IV

- 5 3 percent calcium diwaxbenzene sulfonate  
0.15 percent sulfur as phosphorus pentasulfide treated wax olefin  
4.85 percent barium hydroabietyl alcoholate  
Balance—mineral lubricating oil

10 Other formulations were compounded employing other detergents and corrosion inhibitors and in differing proportions as follows:

## V

- 15 3 percent calcium diwaxbenzene sulfonate  
0.25 percent sulfur as sodium hydroxide neutralized phosphorus pentasulfide treated wax olefin  
4.6 percent barium hydroabietyl alcoholate  
Balance—mineral lubricating oil

## VI

- 20 3 percent barium diwaxbenzene sulfonate  
0.27 percent sulfur as sulfurized terpene  
4.6 percent barium hydroabietyl alcoholate  
Balance—mineral lubricating oil

## VII

- 25 3 percent barium diwaxbenzene sulfonate  
0.12 percent sulfur as zinc dithiophosphate  
4.6 percent barium hydroabietyl alcoholate  
Balance—mineral lubricating oil

## VIII

- 30 3 percent barium diwaxbenzene sulfonate  
0.25 percent sulfur as sulfurized wax olefin  
4.6 percent barium hydroabietyl alcoholate  
Balance—mineral lubricating oil

35 For comparison purposes the following formulations not containing the barium hydroabietyl alcoholate were compounded:

## IX

- 40 2.5 percent calcium diwaxbenzene sulfonate  
0.15 percent sulfur as phosphorus pentasulfide treated wax olefin  
Balance—mineral lubricating oil

## X

- 45 50 3 percent calcium diwaxbenzene sulfonate  
0.15 percent sulfur as phosphorus pentasulfide treated wax olefin  
Balance—mineral lubricating oil

## XI

- 55 6 percent calcium diwaxbenzene sulfonate  
3 percent barium diwaxbenzene sulfonate  
0.15 percent sulfur as phosphorus pentasulfide treated wax olefin  
60 Balance—mineral lubricating oil

These several formulations were then subjected to engine tests, the results of which are tabulated below.

The compositions of Examples IV, V, VI, VII, VIII, and IX were subjected to a Cub engine test. This test may be described briefly as follows: A four-cylinder Cub engine is run for 40 hours at 2,500 R. P. M. with 11 brake horsepower output, an oil temperature of 280° F. and a jacket temperature of 200° F. After completion of the run, the parts of the engine are inspected and assigned demerit ratings based on their condition. The lower the demerit rating, the better is the engine condition and the oil performance. A rating below 10 is considered to be excellent and a rating between 10 and 15 is good. The results of this test are shown in Table I.

Table I

| Example No.                                               | Percentage Composition |         |         |         |         |         |
|-----------------------------------------------------------|------------------------|---------|---------|---------|---------|---------|
|                                                           | IV                     | V       | VI      | VII     | VIII    | IX      |
| Calcium diwaxbenzene sulfonate                            | 3                      | 3       |         |         |         | 2.5     |
| Barium diwaxbenzene sulfonate                             |                        |         | 3       | 3       | 3       |         |
| Sulfur as $P_2S_5$ treated wax olefin                     | 0.15                   |         |         |         |         | 0.15    |
| Sulfur as $NaOH$ neutralized- $P_2S_5$ treated wax olefin |                        | 0.25    |         |         |         |         |
| Sulfur as sulfurized terpene                              |                        |         | 0.27    |         |         |         |
| Sulfur as zinc dithiophosphate                            |                        |         |         | 0.12    |         |         |
| Sulfur as sulfurized wax olefin                           |                        |         |         |         | 0.25    |         |
| Barium hydroabietyl alcoholate                            | 4.85                   | 4.6     | 4.6     | 4.6     | 4.6     | None    |
| Mineral lubricating oil                                   | Balance                | Balance | Balance | Balance | Balance | Balance |
| Demerits                                                  | 11                     | 13      | 13      | 11      | 12      | 17      |

While the contrasts here are not so striking as those obtained in the Witte and Caterpillar tests, it will be seen that the lubricating oil compositions show good over-all performance in the engine.

The compositions of Examples I, III, IV, and X were subjected to the Witte test which may be described as follows: Single cylinder Witte engines using a fuel having an extreme sulfur content of 2 percent were run for 50 hours at 1,800 R. P. M. with about 4½-5 brake horsepower output, an oil temperature of about 145° F. and a jacket temperature of 175-180° F. The condition of the pistons is examined upon completion of the runs and assigned ratings indicating that condition. A high rating is poor and a low rating is good. A Witte piston rating below 4 is considered to be excellent. Those between 4 and about 15 are considered to be good to fair and indicate satisfactory performance of the lubricating oils while ratings above about 20 indicate unsatisfactory performance. The results of this test are shown in Table II.

Table II

| Example No.                           | Percentage Composition |         |         |         |
|---------------------------------------|------------------------|---------|---------|---------|
|                                       | I                      | III     | IV      | X       |
| Calcium diwaxbenzene sulfonate        | 3                      | 3       | 3       | 3       |
| Sulfur as $P_2S_5$ treated wax olefin | 0.15                   | 0.15    | 0.15    | 0.15    |
| Barium hydroabietyl alcoholate        | 3.58                   | 4.21    | 4.85    | None    |
| Mineral lubricating oil               | Balance                | Balance | Balance | Balance |
| Witte Piston Rating                   | 7                      | 10      | 8.5     | 56-57   |

The materials used in these test runs differ only in barium hydroabietyl alcoholate content. It is seen that the presence of the alcoholate materially improves the engine performance as compared with lubricating oil compositions containing no alcoholate.

Compositions of Examples II and XI were subjected to a 120-hour Caterpillar run with 2 percent sulfur fuel. This test is conducted in a single cylinder Caterpillar diesel engine at 1,000 R. P. M. with approximately 20-brake horsepower output, an oil temperature of 145° F. and a jacket temperature of 175-180° F. At the end of the test run, the parts of the engine are inspected and given a demerit rating based on the condition observed. A demerit rating of zero represents a condition wherein there are no deposits and a demerit rating of ten represents the maximum deposit that can be formed. Consequently, low demerit ratings indicate better engine conditions and hence a better performance of the oil in the engine. The results of this test are shown in Table III.

Table III

| Example No.                           | Percentage Composition |         |
|---------------------------------------|------------------------|---------|
|                                       | II                     | XI      |
| Calcium diwaxbenzene sulfonate        | 3                      | 6       |
| Barium diwaxbenzene sulfonate         | 0.15                   | 3       |
| Sulfur as $P_2S_5$ treated wax olefin | 3.93                   | 0.15    |
| Barium hydroabietyl alcoholate        | Balance                | None    |
| Mineral lubricating oil               |                        | Balance |
| Piston Demerits                       | 1.0                    | 7.0     |

It will accordingly be seen that the rating of the lubricating composition containing barium hydroabietyl alcoholate indicates good performance in this test.

The lubricating oil portion of the blends of this invention are preferably the so-called mineral or hydrocarbon oils but may also consist of wholly or contain in part certain fatty oils including corn oil, soybean oil, lard oil, and the like. The blends may likewise contain volatized oils or synthetic oils of lubricating viscosity. Mineral oil is meant to include oils refined from any of the various crude oils refined by any of the usual refining processes including distillation, solvent extraction, acid treatment, clay treatment, dewaxing, and the like.

It will be understood that in addition to the ingredients in the above recited formations, small amounts of other materials, all of which are conventional in this field, may be added as necessary and desired. These include anti-foaming agents, pour-point depressants, material to improve the oiliness of the composition, and the like.

It is apparent that many modifications and variations of the invention as hereinbefore set forth may be made without departing from the spirit and scope thereof. The examples given are by way of illustration only and the invention is limited only by the terms of the appended claims.

I claim:

1. A lubricating composition comprising from about 2 to 5% of an oil soluble calcium diwaxbenzene sulfonate, at least 0.15 percent sulfur as phosphorus penta sulfide treated wax olefin, from about 3 to 6% of a product obtained by reacting a hydroabietyl alcohol wherein said alcohol comprises a mixture of hydrogenated abietyl alcohols containing a non-alcohol fraction amounting to about 13 to 15 percent and the alcohol fraction comprising about 15 percent dehydroabietyl alcohol, about 40 percent dihydroabietyl alcohol and about 45 percent tetrahydroabietyl alcohol with an amount of barium oxide in excess of that which will react stoichiometrically with said alcohol in a lubricating oil under an inert atmosphere and at a temperature of 205 to 225° C., and the balance a mineral lubricating oil.
2. A lubricating composition comprising from about

2 to 5% of an oil soluble calcium diwaxbenzene sulfonate, from about 0.10 to 0.35% sulfur as sulfurized wax olefin, from about 3 to 6% of a product obtained by reacting a hydroabietyl alcohol wherein said alcohol comprises a mixture of hydrogenated abietyl alcohols containing a non-alcohol fraction amounting to about 13 to 15 percent and the alcohol fraction comprising about 15 percent dehydroabietyl alcohol, about 40 percent dihydroabietyl alcohol and about 45 percent tetrahydroabietyl alcohol with 10 an amount of barium oxide in excess of that which will react stoichiometrically with said alcohol in a lubricating

oil under an inert atmosphere and at a temperature of 205 to 225° C., and the balance a mineral lubricating oil.

## References Cited in the file of this patent

## UNITED STATES PATENTS

|              |                  |               |
|--------------|------------------|---------------|
| 2,057,212    | Shoemaker et al. | Oct. 13, 1936 |
| 2,341,565    | Lyman            | Feb. 15, 1944 |
| 2,419,360    | McNab            | Apr. 22, 1947 |
| 10 2,421,004 | Berger           | May 27, 1947  |
| 2,546,552    | Loane            | Mar. 27, 1951 |
| 2,629,693    | Barton et al.    | Feb. 24, 1952 |